

## UNITED STATES PATENT OFFICE

2,214,483

## PHOTOGRAPHIC COLOR PICTURE

Wilhelm Schneider and Hermann Lohaus, Dessau, Germany, assignors, by mesne assignments, to General Aniline & Film Corporation, New York, N. Y., a corporation of Delaware

No Drawing. Application April 3, 1939, Serial No. 265,758. In Germany April 9, 1938

8 Claims. (Cl. 95—6)

Our present invention relates to the manufacture of photographic color pictures.

It is known that photographic color pictures can be produced with the aid of color development by introducing into the developer or into the photographic layer a color former which condenses with certain developer substances to produce a color on the silver image. As dyestuff formers for color development there have been proposed among others aliphatic and aromatic acid methylene compounds, for example ethyl-acetoacetate and its derivatives, ethylbenzoyl-acetate, pyrazolones or the like.

It is one object of our invention to provide a process of the kind in question in which there are used for color development pyroracemic acids and derivatives of pyroracemic acids in which the methyl group contains as a substituent a radicle of aliphatic, isocyclic or heterocyclic nature having double linking adjacent to said methyl group. Vinylene groups may be substituted.

A further object of this invention is the provision of compounds having the following general formula



in which  $R_1$  is a radicle of acyclic, isocyclic or heterocyclic nature which has one or more double linkings adjacent to the  $CH_2$ -group and may contain substituents, for instance methyl, carboxyl or the like, and  $R_2$  is carboxyl, a substituted carboxyl,  $CN$  or the like.

Other objects of our invention will become apparent from the following detailed description.

For example the following compounds may be used: oxalocrotonic acid diethyl ester, oxalosorbic acid diethyl ester, phenyl-pyroracemic acid, quinolyl-pyroracemic acid. The color formers may be added either to the photographic developer or to the emulsion. With color developers, for example para-phenylenediamine or a derivative thereof yellow, orange or red dyestuff images are obtained. When the color former is incorporated in the photographic layer it is to be recommended that it should be made fast to diffusion with respect to the binding agent of the layer by the introduction of special groups. For information about such groups the following U. S. Patent Nos. 2,179,238, 2,178,612, 2,186,849, 2,179,244, 2,186,732, 2,186,733, 2,186,851, 186,719, 2,186,852, and application Ser. No. 191,952, filed February 23, 1938, may be consulted.

The group that is to impart fastness to diffusion may be introduced into the molecule of the color

former in the manner described in the foregoing applications by means of the usual chemical methods; or the color former may be made fast to diffusion by polymerization as described in the said applications. The silver halide emulsion containing color formers fast to diffusion may be used in known manner for making photographic single layer or multi-layer material. The emulsion layers may also be made by distributing differently sensitized emulsions having different color formers in the form of small particles on a support.

The color image may be produced in various manners, for example as described in the U. S. Patent Nos. 2,179,228, 2,179,238, 2,186,849, 2,178,612, 2,186,730, and application Ser. No. 111,250, filed November 17, 1936. The image may be produced in the exposed emulsion layer by simple color development or by reversal development as described for example in the U. S. Patent No. 148,731, filed June 17, 1937, and U. S. Patent No. 2,179,234.

In producing black and white pictures with the aid of silver halide emulsion layers produced in accordance with the invention the silver may be removed or may be left in the layer with the dyestuff image.

The following examples illustrate the invention:

Example 1.—To 1 kilo of a silver halide emulsion 5 grams of the sodium salt of phenylpyroracemic acid of the formula



are added and the emulsion is cast to form a layer. The exposed layer yields on development with para-dimethylaminoaniline a yellow dyestuff image.

Example 2.—To 1 kilo of a silver halide emulsion there are added 5 grams of the sodium salt of the oxalocrotonic acid diethyl ester of the formula



and the emulsion is cast to form a layer. The exposed layer yields on development with para-dimethylaminoaniline a yellow dyestuff image.

Example 3.—To 1 kilo of a silver halide emulsion there are added 5 grams of the sodium salt of the oxalosorbic acid diethyl ester of the formula



and the emulsion is cast to form a layer. The exposed layer yields on development with para-

diethylaminoaniline an orange-red dyestuff image.

Example 4.—To 1 kilo of a silver halide emulsion 5 grams of oxalomethylcrotonic acid ethyl ester are added and the emulsion is cast to form a layer. The exposed layer yields on development with para-diethylaminoaniline a reddish yellow dyestuff image.

Example 5.—To 1 kilo of a silver halide emulsion there are added 5 grams of the sodium salt of ortho-nitrophenyl-pyroracemic acid and the emulsion is cast to form a layer. The exposed layer yields on development with para-diethylaminoaniline a red dyestuff image.

Example 6.—To 1 kilo of a silver halide emulsion there are added 5 grams of the sodium salt of para-nitrophenyl-pyroracemic acid and the emulsion is cast to form a layer. The exposed layer yields on development with para-diethylaminoaniline a red dyestuff image.

Example 7.—To 1 kilo of a silver halide emulsion there are added 5 grams of the sodium salt of a 4-hydroxyphenyl-pyroracemic acid and the emulsion is cast to form a layer. The exposed layer yields on development with para-diethylaminoaniline a yellow dyestuff image.

Example 8.—To 1 kilo of a silver halide emulsion there are added 5 grams of the sodium salt of the quinolyl-2-pyroracemic acid and the emulsion is cast to form a layer. The exposed layer yields on development with para-diethylaminoaniline a yellow dyestuff image.

Example 9.—To 1 kilo of a silver halide emulsion there are added 5 grams of quinolyl-4-pyroracemic acid ethyl ester and the emulsion is cast to form a layer. The exposed layer yields on development with para-diethylaminoaniline a yellow dyestuff image.

Example 10.—4-aminophenyl-pyroracemic acid is caused to react in pyridine with stearic acid chloride and the 4-stearoylaminophenyl-racemic acid thus obtained is precipitated by means of dilute acid. 5 grams of this product are added to 1 kilo of a silver halide emulsion and the emulsion is cast to form a layer. The exposed layer yields on development with para-diethylaminoaniline a yellow dyestuff image.

Example 11.—4-aminophenyl-racemic acid is caused to react in pyridine with 4,4'-diphenyl-dicarboxylic acid chloride and the product is precipitated. 5 grams of the product obtained are added to 1 kilo of a silver halide emulsion and the emulsion is cast to form a layer. The exposed emulsion yields on development with para-diethylaminoaniline a yellow dyestuff image.

Example 12.—To 1 kilo of a silver halide emulsion there are added 5 grams of quinoxalyl-2-pyroracemic acid ethyl ester corresponding with the formula



and the emulsion is cast to form a layer. The exposed layer yields on development with para-diethylaminoaniline an orange dyestuff image.

Example 13.—To 1 kilo of a silver halide emulsion there are added 5 grams of 3-methyl-quinoxalyl-2-pyroracemic acid ethyl ester corresponding with the formula



and the emulsion is cast to form a layer. The exposed layer yields on development with para-diethylaminoaniline an orange dyestuff image.

Example 14.—To 1 kilo of a silver halide emulsion there are added 5 grams of benzoxazole-2-pyroracemic acid corresponding with the formula



and the emulsion is cast to form a layer. The exposed layer yields on development with para-diethylaminoaniline an orange dyestuff image.

Example 15.—To 1 kilo of a silver halide emulsion there are added 5 grams of benzthiazole-2-pyroracemic acid corresponding with the formula



and the emulsion is cast to form a layer. The exposed layer yields on development with para-diethylaminoaniline an orange dyestuff image.

We claim:

1. In a process of producing a photographic color picture by dyestuff forming development, the improvement which comprises causing as the dyestuff former a derivative of the pyroracemic acid, at least the methyl group of said acid being substituted by an organic radicle having an unsaturated double bond in a position adjacent to the carbon atom of said methyl group, to react with the oxidation product of an aromatic developer.

2. In a process of producing a photographic color picture by dyestuff forming development, the improvement which comprises causing as the dyestuff former a compound corresponding with the following general formula:  $R_1-CH_2-CO-R_2$ , in which  $R_1$  is a radicle selected from the class consisting of an aliphatic radicle, an isocyclic radicle and a heterocyclic radicle, said radicle having an unsaturated double bond adjacent to said  $CH_2$ -group,  $R_2$  is a radicle selected from the class consisting of carboxyl, substituted carboxyl, and  $CN$ , to react with the oxidation product of an aromatic developer.

3. In a process of producing a photographic color picture by dyestuff forming development, the improvement which comprises developing the exposed photographic silver halide emulsion with an aromatic amino developer containing as the dyestuff former a derivative of the pyroracemic acid, at least the methyl group of said acid being substituted by an organic radicle having an unsaturated double bond in a position adjacent to the carbon atom of said methyl group.

4. In a process of producing a photographic color picture by dyestuff forming development, the improvement which comprises exposing a photographic silver halide emulsion containing as the dyestuff former a derivative of the pyroracemic acid, at least the methyl group of said acid being substituted by an organic radicle having an unsaturated double bond in a position adjacent to the carbon atom of said methyl group, and developing said emulsion with an aromatic amino developer.

5. In a process of producing a photographic color picture by dyestuff forming development, the improvement which comprises exposing a photographic silver halide emulsion containing as the dyestuff former a derivative of the py-

5 roracemic acid, at least the methyl group of said acid being substituted by an organic radicle having an unsaturated double bond in a position adjacent to the carbon atom of said methyl group, said derivative containing a radicle imparting thereto fastness to diffusion with respect to the binding agent of said emulsion, and developing said emulsion with an aromatic amino developer.

6. Silver halide emulsion for color photography 10 comprising a derivative of the pyroracemic acid, at least the methyl group of said acid being substituted by an organic radicle having an unsaturated double bond in a position adjacent to the carbon atom of said methyl group, said derivative containing a radicle imparting thereto fastness to diffusion with respect to the binding agent of said emulsion.

7. A dyestuff forming developer comprising an aqueous solution containing an aromatic amino 20 developing agent and a derivative of the pyroracemic acid, at least the methyl group of said acid being substituted by an organic radicle having an unsaturated double bond in a position

adjacent to the carbon atom of said methyl group.

8. A silver halide emulsion for color photography containing as a color-forming development component a derivative of pyroracemic acid 5 of the following general formula



10 wherein  $R_1$  is an organic radicle, having an unsaturated double bond in a position adjacent to the



15

group,  $R_2$  being a radicle selected from the group consisting of carboxyl, substituted carboxyl, and the CN group, said color-forming development component containing in its molecule a radicle which imparts thereto fastness to diffusion. 20

WILHELM SCHNEIDER.  
HERMANN LOHAUS.